# EUROPEAN PATENT SPECIFICATION

(11) **EP 0 476 230 B1**
(45) Date of publication and mention of the grant of the patent: **18.12.1996**
(21) Application number: 91108241.0
(22) Date of filing: 22.05.1991
(51) Int. Cl.: D21C 3/02, D21C 7/00

(54) **Extended kraft cooking with white liquor added to wash circulation**
Verlängertes Kraftkochen mit dem Waschkreislauf zugefügter Weisslauge
Cuisson kraft complète avec lessive blanche ajoutée à la circulation de lavage

(30) Priority: 17.09.1990 US 583043
(43) Date of publication of application: 25.03.1992
(73) Proprietor: Kamyr, Inc., Glens Falls, New York 12801-3686 (US)
(72) Inventor: Stromberg, Bertil Kamyr Inc., New York 12801-3686 (US); Jiang, Jian Kamyr Inc., New York 12801-3686 (US); Laakso, Richard Kamyr, Inc., New York 12801-3686 (US); Phillips, Joseph Kamyr Center, New York 12801-3686 (US); Greenwood, Brian Kamyr Center, New York 12801-3686 (US); Prough, James Kamyr Inc., New York 12801-3686 (US)
(74) Representative: UEXKÜLL & STOLBERG

(56) References cited:
- EP-A- 0 407 370
- US-A- 3 215 588
- US-A- 3 427 218

## Description

### BACKGROUND AND SUMMARY OF THE INVENTION

In recent years, great strides have been made in improving the continuous kraft pulping of comminuted cellulosic fibrous material (e.g. wood chips) to produce kraft pulp. In conventional continuous digestion systems, the white liquor was added only to the recirculation loop between the digester and other components, and/or into an impregnation vessel. However, in about 1983, it was recognized the increased bleach brightness potential and savings in bleaching chemicals could be utilized if kraft white liquor were added in a number of places in the process, including (and most importantly) in a central recirculation loop within the continuous upright digester. Black liquor was withdrawn from screens between the top and central portion of the digester, meaning that for a part of the cooking zone the kraft white liquor flowed countercurrently to the cellulosic material.

While the improved process and system as described above -- marketed commercially by Kaymr, Inc. of Glens Falls, New York and Kaymr AB of Karlstad, Sweden under the trademark "MCC" and described in an article by W. Eric Wiley, "Pulp quality up, chemical costs down with MCC" in PIMA magazine, May 1987, -- has resulted in vast improvements in the many commercial installations in which it has been used since its commercial introduction in 1985, it is desirable to effect still further improvements in continuous kraft pulping.

The invention relates to a method as claimed in claim 1 and to an apparatus as claimed in claim 9.

It is the primary object of the present invention to improve conventional continuous kraft pulping processes. This and other aspects of the invention will become clear from an inspection of the detailed description of the invention and from the appended claims.

### BRIEF DESCRIPTION OF THE DRAWINGS

FIGURE 1 is a side schematic view showing an exemplary kraft pulping apparatus according to the present invention;
FIGURE 2 is a graphical representation plotting viscosity versus Kappa Number when comparing the invention to prior art continuous kraft pulping procedures; and
FIGURE 3 is a representation like that of Figure 2 plotting the viscosity/Kappa Number ratio versus Kappa Number.

### DETAILED DESCRIPTION OF THE DRAWINGS

An exemplary apparatus for kraft pulping according to the invention is illustrated in Figure 1. Entirely standard components include a chips bin 10 for receiving a feed of chips 11 or like cellulosic comminuted fibrous material. From the chips bin 10, the material goes to a horizontal steaming vessel 12, and a vertical conduit 13, kraft white liquor from the source 14 being added to the material in the conduit 13 to slurry the material as it is fed to the high pressure feeder 15. From the high pressure feeder 15 the material entrained in kraft white liquor passes to an optional impregnation vessel 16, and then in line 17 to the top 18 of a continuous digester 19. At the top of the digester 19 there is a liquid/material separation device 20, which preferably comprises a plurality of bull screens with switching withdrawal from the screens, or the like. The digester 19 also includes a central portion 21 and a bottom 22.

At a portion of the digester 19 between the top 18 and the central portion 21 thereof one or more screens 23, and conduit 24, are provided as means for extracting black liquor from the digester 19. The black liquor is typically passed in conduit 24 to a series of flash tanks 25, as is conventional. At the central portion 21 of the digester 19, withdrawal screens 27 are also provided, being connected by a withdrawal conduit to a pump 28 and a heater 29 for re-introduction of the withdrawn liquid at point 30 of a re-introduction conduit, the point 30 typically being slightly above the screens 27. At the bottom 22 of the digester, kraft pulp is withdrawn in conduit 33 (a scraper or like conventional components can also be utilized), and wash liquor from source 34 is added in introduction conduit 35.

Adjacent the bottom of the digester 19 a wash screen (one or more rows) 37 is provided, liquid being withdrawn therethrough in a withdrawal conduit under the influence of pump 38, and then passing through heater 39 into a re-introduction conduit to be introduced at point 40 just above the screen 37. From the point 40 up to the screens 23, liquid flows countercurrently to the material -- as designated by arrows 42 -- while above the screens 23 it flows cocurrently.

What has been described so far, and including a main conduit 44 for adding kraft white liquor in conduit 45 to the first recirculation loop at digester central portion 21, is conventional in the Kamyr MCC™ system. According to the present invention, a conduit 46 is provided for interconnecting the main conduit 44 to the withdrawal conduit in the second, wash, recirculation loop provided by elements 37 through 40.

In the practice of the present invention, sufficient kraft white liquor is added in conduit 46 so as to achieve significantly enhanced viscosity and strength properties of the pulp produced compared to the practice of the same method without the introduction of kraft white liquor in conduit 46. For example, the amount of kraft white liquor added in conduit 46 is at least about 5% of the total amount of kraft liquor utilized to effect kraft pulping, and typically is about 10-20% (e.g. about 15%). Kraft white liquor preferably is also added -- as is known per se -- in conduit 45 in addition to conduit 46, the amount added in conduit 45 being at least about 10%, and preferably about 10-20%.

The apparatus of Figure 1 also includes a recirculation loop at a central portion of the impregnation vessel 16, including screen 48, withdrawal conduit 49, pump 50, and re-introduction conduit/point 51. Kraft white liquor from source 14 also is preferably added as indicated by lines or points 52, 53, 54 to the recirculation loop in the impregnation vessel 16, and to the recirculation conduits from the digester to the impregnation vessel 16, and from the impregnation vessel 16 to the high pressure feeder 15. Normally the majority of the white liquor used in the conventional continuous kraft pulping process is added at the points or conduits 52 - 54.

Graphical representations of some of the improved results achieved according to the present invention are illustrated in Figures 2 and 3. As can be seen in Figure 2, viscosity is plotted against Kappa Number for three major different processes. The first procedure -- illustrated by line 55 -- is conventional continuous kraft cooking. The second procedure -- illustrated by line 56 -- is for the Kamyr MCC™ system and process. The data points 57 illustrate results achieved by practicing the present invention. In the practice of the procedures resulting in the data plotted in Figure 2, all parameters were maintained essentially the same except for the addition of kraft white liquor, and the temperature in the wash zone according to the invention was raised to about 140-175°C, compared to about 125-130°C for conventional kraft cooking and Kamyr's MCC™ process. The conditions resulting in the plots in Figures 2 and 3 are set forth in the following table:

**TABLE I**

| Cook Type | Conventional | MCC™ | Invention |
|---|---|---|---|
| Presteaming | | | |
| | | | |
| Time, min | 5 | 5 | 5 |
| Temp., °C | 110 | 110 | 110 |
| | | | |
| Impregnation, L/W = 4 | | | |
| | | | |
| WL to feed, % as NaOH on wood (% of total WL used) | 16.2 (90%) | 11.7 (65%) | 10.8 (60%) |
| Time, min | 30 | 30 | 30 |
| Temp., °C | 120 | 120 | 120 |
| | | | |
| Co-Current Stage | | | |
| | | | |
| WL to BC, % as NaOH on wood (% of total WL used) | 1.8 (10%) | 3.6 (20%) | 2.7 (15%) |
| Max. temp., °C | 170 | 170 | 165 |
| Total time, min. | 90 | 45 | 45 |
| | | | |
| Central Stage | | | |
| | | | |
| WL, % as NaOH on wood (% of total WL used) | - | 2.7 (15%) | 1.8 (10%) |
| Max. temp., °C | - | 170 | 165 |
| Time, min. | - | 60 | 60 |
| | | | |
| Wash Stage | | | |
| | | | |
| WL, % as NaOH on wood (% of total WL used) | - | - | 2.7 (15%) |
| Max. temp., °C | 135 | 135 | 165 |
| Time, min. | 180 | 180 | 180 |

Conditions for all cooks were targeted at total EA (WL) addition of 18% NaOH based on wood.

In tests of the conventional kraft process which resulted in graph line 55, white liquor was added only at points 53 and 54. In the testing that resulted in graph line 56, white liquor was also added in conduit 45. In the practice of the present invention -- resulting in data points 57 -- about 15% of the kraft white liquor necessary to effect kraft pulping was added in conduit 46, with about 10% in conduit 45, and the rest in 53 and 54.

In the practice of the invention, the addition of white liquor at 53 is normally about 50-60% of the total white liquor added, and about 10-20% at 54 (with about 10-20% at 45, and 5-20% at 46).

Figure 3 graphically illustrates the same test results as Figure 2, only the viscosity/Kappa Number ratio is plotted against Kappa Number. The graphical representation 60 is attained during conventional kraft cooking, the graphical representation 61 during the practice of the Kamyr MCC™ process and system, and the data points 62 in the practice of the present invention.

As can be seen from both Figures 2 and 3, the viscosity of the plots produced according to the invention is at least 30% greater than for the best prior art system (MCC™), and can be expected to be at least 20% greater.

According to the present invention not only does the viscosity of the final pulp produced increase, the strength properties (tear, tensile, and burst) are also increased for a given Kappa Number. Further, unexpectedly, the entire digester becomes easier to operate. The easier operation of the digester alone is enough to warrant utilization of the method according to the invention.

Advantageous results are achieved according to the invention whether or not an impregnation vessel 16 is provided, and most of the advantageous results according to the invention are achieved whether or not white liquor is added in conduit 45. However, optimum results are obtained when utilizing an impregnation vessel 16, and also adding white liquor in conduit 45.

It will thus be seen that according to the present invention an improved method and apparatus for the continuous kraft pulping of cellulosic material is provided. While the invention has been herein shown and described in what is presently conceived to be the most practical and preferred embodiment thereof, the same principles can be applied to a single vessel hydraulic digester and either one or two vessel steam/liquor phase digesters.

## Claims

1. A method of continuously kraft pulping comminuted cellulosic fibrous material using an upright digester (19) having top (18), bottom (22), and central (21) portions, comprising the step of:
(a) passing comminuted cellulosic fibrous material entrained in kraft white liquor into the top of the digester; (b) extracting black liquor from at least one screen (23) between the top and the central portion of the digester; (c) at a central portion of the digester withdrawing and recirculating liquid in a first recirculation loop (28, 29), the liquor recirculated into the digester in part passing upwardly therein countercurrent to the material flow; (d) adding wash liquid (34) at the bottom of the digester; (e) withdrawing kraft pulp from the bottom of the digester;
(f) adjacent the bottom of the digester withdrawing and recirculating liquid in a second, wash, recirculation loop (38, 39); (g) adding white liquor to the first recirculation loop; and (h) adding kraft white liquor (14) to said second recirculation loop, the liquor recirculated into the digester in part passing upwardly therein countercurrent to the material flow; and the amount of white liquor added in said second recirculation loop being sufficient to increase the viscosity and strength properties of the pulp produced compared to the practice of the same method with the same material, Kappa Number, and other parameters only without step (h).

2. A method as recited in claim 1 further characterized in that step (h) is practiced so that about 5-20% of the total amount of kraft white liquor utilized to effect kraft pulping is added during the practice of step (h).

3. A method as recited in claim 1 further characterized in that steps (a)- (f) are practiced so that the majority of kraft white liquor is added in step (a) and at least 5% of the total kraft liquor utilized for kraft cooking as added in step (h), and the temperature in step (h) is about 140-175°C.

4. A method as recited in claim 1 further utilizing an impregnation vessel (16), and a conduit (17) connected between the impregnation vessel and the digester, and further characterized in that step (a) is practiced by adding kraft white liquor (14) to the conduit and impregnation vessel, and so that the majority of the kraft white liquor added is added in the conduit and the impregnation vessel, about 5-20% of the kraft white liquor utilized to effect kraft cooking is added in step (h), and about 10-20% of the kraft white liquor utilized is added in step (g).

5. A method as recited in claim 1 further characterized in that in both the first and second circulation loops the liquid is pumped (via 28, 38) and heated (via 29, 39) before being reintroduced into the digester, and further characterized in that steps (g) and (h) are practiced by introducing the kraft white liquor prior to (at 45, 46) the pumping and heating of the recirculated liquid in the recirculation loop.

6. A method as recited in claim 1 further characterized in that step (h) is practiced so as to increase the viscosity of the kraft pulp produced, at a given Kappa Number, by at least about 20% compared to pulp produced by the practice of only steps (a)-(g) above.

7. A method as recited in claim 6 further characterized by the step of maintaining the temperature in the wash zone at about 140-175°C.

8. A method as recited in claim 1 further characterized in that step (h) is practiced so as to increase the viscosity of the kraft pulp produced, at a given Kappa Number, by at least about 30% compared to pulp produced by the practice of only steps (a)-(g) above, by maintaining the temperature in the wash zone at about 140-175°C and adding about 15% kraft white liquor in conduit (46), about 10% in conduit (45) and the rest in conduits (53 & 54).

9. Apparatus for continuously kraft pulping comminuted cellulosic fibrous material comprising:
an upright digester vessel (19), having top (18), bottom (22), and central (21) portions; means (17) for introducing comminuted cellulosic fibrous material entrained in white liquor into the top of the digester; means (23, 24) for extracting black liquor from at least one screen (23) between the top of the digester and the central portion thereof; at the central portion of the digester, means (27, 28) for withdrawing and recirculating liquid in a first circulation loop; means (34, 35) for adding wash liquid to the bottom of the digester; means (33) for withdrawing kraft pulp from the bottom of the digester;
means (37, 38) adjacent the bottom of the digester, for withdrawing and recirculating liquid in a second, wash, recirculation loop; and means (14, 44, 45) for introducing white liquor into said first recirculation loop;
characterized by means (14, 44, 46) for introducing white liquor into said second recirculation loop.

10. Apparatus as recited in claim 9 further characterized in that each recirculation loop comprises a withdrawal conduit, pump (28, 38), heater (39, 29) and re-introduction conduit (30, 40), and said means for introducing white liquor into each recirculation loop comprises means (45, 46) for introducing the liquor in said withdrawal conduit before the pump and heater.

11. Apparatus as recited in claim 9 further comprising an upright impregnation vessel (16) having a top and a bottom, and a conduit (17) for interconnecting the bottom of the impregnation vessel to the top of the digester and a recirculation loop (54) for recirculating liquid from the top of the digester to the bottom of the impregnation vessel, and at a central portion of the impregnation vessel, means (48-51) for withdrawing and recirculating liquid in a third circulation loop, and means (14, 52) for introducing white liquor into said third recirculation loop.

## Patentansprüche

1. Verfahren zum kontinuierlichen Kraftauslaugen von zerkleinertem Zellulosefasermaterial mit einem aufrechtstehenden Zellulosekocher (19) mit einem Deckel (18), einem Boden (22) und Rumpfabschnitten (21), mit den Schritten:
(a) Einfüllen von zerkleinertem Zellulosefasermaterial, das in Kraft-Weißlauge mitgeführt wird, in den Deckel des Zellstoffkochers; (b) Abscheiden von Ablauge aus mindestens einem Filter (23) zwischen dem Deckel und dem Rumpfabschnitt des Zellstoffkochers; (c) Entziehen und Umwälzen von Flüssigkeit in einem Rumpfabschnitt des Zellstoffkochers in einer ersten Umwälzschleife (28, 29), wobei die in den Zellstoffkocher zurückfließende Lauge teilweise darin aufwärts, gegenläufig zum Materialstrom fließt; (d) Hinzufügen von Waschflüssigkeit (34) in den Boden des Zellstoffkochers; (e) Entziehen von Kraftzellstoff aus dem Boden des Zellstoffkochers; (f) Abziehen und Umwälzen von Flüssigkeit nahe dem Boden des Zellstoffkochers in einer zweiten Wasch- und Umwälzschleife (38, 39); (g) Hinzufügen von Weißlauge zur ersten Umwälzschleife; und (h) Hinzufügen von Kraft-Weißlauge (14) zur zweiten Umwälzschleife, wobei die in den Zellstoffkocher zurückfließende Lauge teilweise darin aufwärts, gegenläufig zum Materialstrom fließt; und wobei die Menge von Weißlauge, die in der zweiten Umwälzschleife hinzugefügt wird, ausreichend ist, um die Viskosität und die Festigkeitseigenschaften des erzeugten Zellstoffs im Vergleich zur Anwendung des gleichen Verfahrens mit dem gleichen Material, der gleichen Kappazahl, und anderen Parametern nur ohne den Schritt (h) zu steigern.

2. Verfahren nach Anspruch 1, ferner **dadurch gekennzeichnet**, daß der Schritt (h) so ausgeführt ist, daß ca. 5 bis 20% der Gesamtmenge der Kraft-Weißlauge, die für das Kraftauslaugen verwendet wird, während der Ausführung des Schritts (h) hinzugefügt wird.

3. Verfahren nach Anspruch 1, ferner **dadurch gekennzeichnet**, daß die Schritte (a) bis (f) so ausgeführt werden, daß der Großteil der Kraft-Weißlauge im Schritt (a) und mindestens 5% der gesamten Kraftlauge, die zum Kraftkochen verwendet wird, im Schritt (h) hinzugefügt wird und die Temperatur im Schritt (h) ungefähr 140 bis 175°C beträgt.

4. Verfahren nach Anspruch 1, ferner unter Verwendung eines Imprägnierkessels (16) und einer Leitung (17), die zwischen den Imprägnierkessel und den Zellstoffkocher gelegt ist, und ferner **dadurch gekennzeichnet**, daß der Schritt (a) durch Einspeisen von Kraft-Weißlauge (14) in die Leitung und in den Imprägnierkessel ausgeführt und der Großteil der eingespeisten Kraft-Weißlauge in die Leitung und in den Imprägnierkessel eingespeist wird, wobei ungefähr 5 bis 20% der Kraft-Weißlauge, die für das Kraftkochen verwendet wird, in dem Schritt (h) und ungefähr 10 bis 20% der verwendeten Kraft-Weißlauge in dem Schritt (g) hinzugefügt werden.

5. Verfahren nach Anspruch 1, ferner **dadurch gekennzeichnet**, daß sowohl in der ersten als auch in der zweiten Umwälzschleife die Flüssigkeit gepumpt (durch 28, 38) und aufgeheizt (durch 29, 39) wird, bevor sie in den Zellstoffkocher zurückgeführt wird, und ferner **dadurch gekennzeichnet**, daß die Schritte (g) und (h) durch Einleiten der Kraft-Weißlauge vor dem Pumpen (bei 45, 46) und Aufheizen der zurückfließenden Flüssigkeit in die Umwälzschleife ausgeführt werden.

6. Verfahren nach Anspruch 1, ferner **dadurch gekennzeichnet**, daß der Schritt (h) so ausgeführt ist, daß die Viskosität des erzeugten Kraftzellstoffs bei einer gegebenen Kappazahl um mindestens ungefähr 20% im Vergleich zu dem Zellstoff gesteigert wird, der nur durch die Anwendung der obigen Schritte (a) bis (g) erzeugt wird.

7. Verfahren nach Anspruch 6, ferner **gekennzeichnet** durch den Schritt des Beibehaltens der Temperatur in der Waschzone bei ungefähr 140 bis 175°C.

8. Verfahren nach Anspruch 1, ferner **dadurch gekennzeichnet**, daß der Schritt (h) so ausgeführt ist, daß die Viskosität des erzeugten Kraftzellstoffs bei einer gegebenen Kappazahl um mindestens ungefähr 30% gesteigert wird im Vergleich zu dem Zellstoff, der nur durch die Anwendung der obigen Schritte (a) bis (g) erzeugt wird, unter Beibehaltung der Temperatur in der Waschzone bei ungefähr 140 bis 175°C und Hinzufügen von ungefähr 15% Kraft-Weißlauge in die Leitung (46), ungefähr 10% in die Leitung (45) und dem Rest in die Leitung (53 und 54).

9. Vorrichtung zum kontinuierlichen Kraftauslaugen von zerkleinertem Zellulosefasermaterial mit:
einem aufrechtstehenden Zellstoffkochkessel (19) mit einem Deckel (18), einem Boden (22) und Rumpfabschnitten (21); Mitteln (17) zum Einführen von zerkleinertem Zellulosefasermaterial, das in Weißlauge mitgeführt wird, in den Deckel des Zellstoffkochers; Mitteln (23, 24) zum Abscheiden von Ablauge aus mindestens einem Filter (23) zwischen dem Deckel des Zellstoffkochers und dem Rumpfabschnitt; Mitteln (27, 28) an dem Rumpfabschnitt des Zellstoffkochers zum Entziehen und Umwälzen von Flüssigkeit in einer ersten Umwälzschleife; Mitteln (34, 35) zum Hinzufügen von Waschflüssigkeit an dem Boden des Zellstoffkochers; Mitteln (33) zum Entziehen von Kraftzellstoff aus dem Boden des Zellstoffkochers; Mitteln (37, 38) neben dem Boden des Zellstoffkochers zum Entziehen und Umwälzen von Lauge in einer zweiten Wasch- und Umwälzschleife; und Mitteln (14, 44, 45) zum Einführen von Weißlauge in die erste Umwälzschleife;
**gekennzeichnet** durch Mittel (14, 44, 46) zum Einführen von Weißlauge in die zweite Umwälzschleife.

10. Vorrichtung nach Anspruch 9, ferner **dadurch gekennzeichnet**, daß jede Umwälzschleife eine Entnahmeleitung, eine Pumpe (28, 38), eine Heizung (39, 29) und Wiedereinlaßleitungen (30, 40) aufweist, und daß das Mittel zum Einleiten von Weißlauge in jede Umwälzschleife ein Mittel (45, 46) zum Einleiten der Lauge in die Entnahmeleitung vor der Pumpe und der Heizung aufweist.

11. Vorrichtung nach Anspruch 9, ferner mit einem aufrechtstehenden Imprägnierkessel (16) mit einem Deckel und einem Boden und mit einer Leitung (17) zum Verbinden des Bodens des Imprägnierkessels mit dem Deckel des Zellstoffkochers und mit einer Umwälzschleife (54) zum Umwälzen von Lauge aus dem Deckel des Zellstoffkochers in den Boden des Imprägnierkessels und mit Mitteln (48 bis 51) in einem Rumpfabschnitt des Imprägnierkessels zum Abziehen und Umwälzen von Lauge in einer dritten Umwälzschleife, und mit Mitteln (14, 52) zum Einleiten von Weißlauge in die dritte Umwälzschleife.

## Revendications

1. Procédé de réduction continue en pulpe kraft de matière fibreuse cellulosique réduite en poudre utilisant un lessiveur vertical (19) ayant des portions de dessus (18), de fond (22) et des portions centrales (21), comprenant les étapes de :
(a) passage de la matière fibreuse cellulosique réduite en poudre entraînée dans de la lessive fraîche kraft dans le dessus du lessiveur,
(b) extraction de la lessive noire d'au moins un crible (23) entre la portion de dessus et la portion centrale du lessiveur,
(c) à une portion du lessiveur, retrait et recirculation du liquide dans une première boucle de recirculation (28, 29), la lessive recirculée dans le lessiveur passant en partie vers le haut à l'intérieur à contre-courant du flux de matière,
(d) addition de liquide de lavage (34) au fond du lessiveur,
(e) retrait de la pulpe kraft du fond du lessiveur,
(f) de manière adjacente au fond du lessiveur, retrait et recirculation du liquide dans une seconde boucle de lavage et recirculation (38, 39),
(g) addition de lessive blanche à la première boucle de recirculation et
(h) addition de lessive blanche kraft à ladite seconde boucle de recirculation, la lessive recirculée dans le lessiveur passant en partie vers le haut à l'intérieur à contre-courant du flux de matière et la quantité de lessive blanche ajoutée dans ladite seconde boucle de recirculation étant suffisante pour augmenter les propriétés de viscosité et de résistance de la pulpe produite comparée à la pratique du même procédé avec la même matière, le même indice Kappa et d'autres paramètres seulement sans l'étape (h).

2. Procédé selon la revendication 1, de plus caractérisé en ce que l'étape (h) est pratiquée de telle manière qu'environ 5 à 20 % de la quantité totale de lessive blanche kraft utilisée pour effectuée la réduction en pulpe kraft sont ajoutés pendant la pratique de l'étape (h).

3. Procédé selon la revendication 1, de plus caractérisé en ce que les étapes (a) - (f) sont pratiquées de telle manière que la majorité de la lessive blanche kraft est ajoutée dans l'étape (a) et qu'au moins 5 % de la lessive kraft totale utilisée pour la cuisson kraft, telle qu'utilisée dans l'étape (h), et la température dans l'étape (h) est d'environ 175° C.

4. Procédé selon la revendication 1, utilisant de plus un récipient d'imprégnation (16) et un conduit (17) relié entre le récipient d'imprégnation et le lessiveur, et de plus caractérisé en ce que l'étape (a) est pratiquée en ajoutant de la lessive blanche kraft (14) au conduit et au récipient d'imprégnation et de telle manière que la majorité de la lessive blanche kraft ajoutée est ajoutée dans le conduit et le récipient d'imprégnation, environ 5 à 20 % de la lessive blanche kraft utilisée pour effectuer la cuisson kraft sont ajoutés dans l'étape (h) et environ 10 à 20 % de la lessive blanche kraft utilisée sont utilisés dans l'étape (g).

5. Procédé selon la revendication 1, de plus caractérisé en ce que le liquide est pompé (par 28, 38) et réchauffé (par 29, 39) dans les deux boucles de recirculation, la première et la seconde, avant d'être réfntroduit dans le lessiveur et caractérisé de plus en ce que les étapes (g) et (h) sont pratiquées en introduisant la lessive blanche kraft avant (à 45, 46) le pompage et le chauffage du liquide recirculé dans la boucle de recirculation.

6. Procédé selon la revendication 1, de plus caractérisé en ce que l'étape (h) est pratiquée de manière à augmenter la viscosité de la pulpe kraft produite, à un indice Kappa donné, d'au moins environ 20 %, comparée à la pulpe produite par la pratique des seules étapes (a)-(g) ci-dessus.

7. Procédé selon la revendication 6, caractérisé de plus par l'étape de maintien de température dans la zone de lavage à environ 140-175° C.

8. Procédé selon la revendication 1, caractérisé de plus en ce que l'étape (h) est pratiquée de manière à augmenter la viscosité de la pulpe kraft produite, à un indice Kappa donné, d'au moins environ 30 %, comparée à la pulpe produite par la pratique des seules étapes (a)-(g) ci-dessus, en maintenant la température dans la zone de lavage à environ 140-175° C et en ajoutant environ 15 % de lessive blanche kraft dans le conduit (46), environ 10 % dans le conduit (45) et le reste dans les conduits (53 et 54).

9. Appareil pour réduction continue en pulpe kraft de matière fibreuse cellulosique réduite en poudre comprenant :
un récipient lessiveur vertical (19), ayant des portions de dessus (18), de fond (22) et centrales (21), des moyens (17) pour introduire la matière fibreuse cellulosique réduite en poudre entraînée dans la lessive blanche dans le dessus du lessiveur, des moyens (23, 24) pour extraire la lessive noire d'au moins un crible (23) entre le dessus du lessiveur et la portion centrale de celui-ci, dans la portion centrale du lessiveur des moyens (27, 28) pour retirer et recirculer le liquide dans une première boucle de circulation, des moyens (34, 35) pour ajouter du liquide de lavage au fond du lessiveur, des moyens (33) pour retirer la pulpe kraft du fond du lessiveur, des moyens (37, 38) adjacents au fond du lessiveur pour retirer et recirculer du liquide dans une seconde boucle de lavage et de recirculation et des moyens (14, 44, 45) pour introduire la lessive blanche dans ladite première boucle de recirculation, caractérisé par des moyens (14, 44, 46) pour introduire la lessive blanche dans ladite seconde boucle de recirculation.

10. Appareil selon la revendication 9, de plus caractérisé en ce que chaque boucle de recirculation comprend un conduit de retrait, une pompe (28, 38), un appareil de chauffage (39, 29) et un conduit de réintroduction (30, 40) et lesdits moyens pour introduire la lessive blanche dans chaque boucle de recirculation comprennent des moyens (45, 46) pour introduire la lessive dans ledit conduit de retrait avant la pompe et l'appareil de chauffage.

11. Appareil selon la revendication 9, comprenant de plus un récipient d'imprégnation vertical (16) ayant un dessus et un fond, et un conduit (17) pour relier le fond du récipient d'imprégnation au dessus du lessiveur, et une boucle de recirculation (54) pour recirculer le liquide du dessus du lessiveur au fond du récipient d'imprégnation, et, à la portion centrale du récipient d'imprégnation, des moyens (48-51) pour retirer et recirculer le liquide dans une troisième boucle de circulation, et des moyens (14, 52) pour introduire la lessive blanche dans ladite troisième boucle de recirculation.
